

1,172,682.

H. L. DOHERTY.  
PROCESS FOR CARBONIZING COAL.  
APPLICATION FILED DEC. 27, 1909.

Patented Feb. 22, 1916.

3 SHEETS—SHEET 1.



Fig. 2.



Witnesses:  
M. J. Marentin  
W. G. Berrymore

Henry L. Doherty, Inspector

By his Attorney Frank S. Young.

1,172,682.

H. L. DOHERTY,  
PROCESS FOR CARBONIZING COAL,  
APPLICATION FILED DEC. 27, 1909.

Patented Feb. 22, 1916.

3 SHEETS—SHEET 2.

Fig. 3.



Fig. 4.



Fig. 5.



Fig. 6.



Witnesses:  
W. J. Doherty  
H. G. Berryman

Henry L. Doherty, Inventor  
By his Attorney Frank S. Young.

1,172,682.

H. L. DOHERTY,  
PROCESS FOR CARBONIZING COAL,  
APPLICATION FILED DEC. 27, 1909.

Patented Feb. 22, 1916.

3 SHEETS—SHEET 3.



FIG. 7.

Witnesses:  
John J. Quinn  
H. G. Berryman

Henry L. Doherty, Inventor  
By his Attorney Frank S. Young.

# UNITED STATES PATENT OFFICE.

HENRY L. DOHERTY, OF NEW YORK, N. Y.

## PROCESS FOR CARBONIZING COAL.

1,172,682.

Specification of Letters Patent. Patented Feb. 22, 1916.

Application filed December 27, 1909. Serial No. 535,036.

To all whom it may concern:

Be it known that I, HENRY L. DOHERTY, a citizen of the United States, and resident of New York city, in the county of New York and State of New York, have invented certain new and useful Improvements in Processes for Carbonizing Coal, of which the following is a specification.

This invention relates to processes for carbonizing coal and particularly to that kind of such processes in which the heat for the carbonization of the coal is supplied to the same by conduction from a bath of molten material.

The object of my invention is the furnishing of a method for carbonizing coal in which the carbonization can be carried on at a uniformly low temperature and yet with a speed much greater than by carbonization in fireclay retorts according to the process at present in use.

Briefly my process consists in circulating a suitable molten material in a closed circuit first through a reheating chamber and then through a carbonizing chamber, feeding crushed coal onto the molten material in the carbonizing chamber, allowing said coal to remain in contact with the molten material in the carbonizing chamber for a sufficient length of time to carbonize the said coal and removing from the carbonizing chamber the gas and coke resulting from the carbonization of the coal.

In the accompanying drawings, Figure 1, is a vertical longitudinal section through the carbonizing chamber on a plane through the line A B of Fig. 2 and A' B' of Fig. 7. Fig. 2 is a horizontal cross-section through the carbonizing and reheating chambers on a plane through the line C D of Fig. 1. Fig. 3, is a vertical longitudinal section through the recuperator on a plane through the line G H of Fig. 7. Fig. 4 is a vertical cross-section of the recuperator on a plane through the line E F of Fig. 7. Fig. 5 is a partial vertical section through the wall separating the reheater and carbonizing chambers, across the connecting passage, showing the device for operating the circulating apparatus. Fig. 6 is a horizontal partial section through the passage connecting the reheater and carbonizer showing a top view of the circulating means. Fig. 7 is a diagrammatic plan of the apparatus.

The apparatus figured, of course, is only one of the many means of carrying out my

process that may be used, and I do not limit myself to this particular design of apparatus.

In the form of apparatus shown, 1, is the carbonizing chamber, 2, the reheater for reheating the material of the molten bath, 3, is the recuperator. The coal to be distilled is fed into the charging hopper, 4, the coal being preferably first crushed to such a size as will pass through a screen of  $\frac{1}{4}$  inch mesh. Reduction to this size is not an imperative requirement of my process but I find that this size is well adapted to give the best results. The larger the size of the coal fragments the longer is the time, that the coal must be allowed to remain in contact with the molten bath. Therefore, I find it preferable in order to increase the speed of operation, to crush the coal, as mentioned, although I do not restrict myself to the use of crushed coal in my process. From 4 the coal is dropped into the feed-box 5 by raising the lever arm 6 which causes the lowering of the charging cone 6'. The bottom of 5 slopes to a narrow slot 7 which is in communication with a cylindrical casing 8 in which works the feed-roll 9.

10 is a slot in the bottom of casing 8 which communicates with the vertical chute 10'; the latter discharging into the interior chamber 11 of carbonizer 1. The feed roll 9 has a shaft, 9', operated by a suitable mechanism 9'', and has longitudinal grooves 9''' on its surface. On causing the shaft 9' to rotate the coal in 5 enters the grooves 9''' as they pass under the slot 7 and falls out of the grooves again as they pass over the discharge slot 10, falling through the chute 10' on to the surface of the bath of molten material 12, in chamber 11. The slot 10 and chute 10' extend across the full width of the carbonizing chamber. The feed roll working fairly tight in the casing 8 shuts off all communication between 11 and 5 thus preventing any loss of gas through 5 and 4 when the latter is opened for the introduction of coal. The coal floats on the surface of the flowing bath or stream of molten material 12 and moves with it to the discharge end of the carbonizing chamber. While resting on the surface of the bath the coal is, of course, subjected to the action of the heat of the molten material, and is therefore, quickly carbonized, its volatile matter distilling off. Since I prefer to use some material having a high co-efficient of conduc-

tivity for the bath and there is always in chamber 11 a weight of the material constituting the bath many times the weight of the coal present at any given time, the distillation takes place with great rapidity, the heat capacity of the bath being very great relative to that of the coal present. I prefer to work with a layer of coal of comparative thinness, advantageously, not exceeding, say  $\frac{1}{4}$ " in thickness, although, of course, this depth of coal may be considerably increased if desired. With the layer of coal restricted to the given thickness the distillation takes place very quickly, not requiring more than about 2 minutes to reach completion. With an increase of thickness of the layer of coal charged, the rate of flow of the bath or stream of molten material must, of course, be materially diminished, since, in this case, the coal of the upper portion of the layer is not in direct contact with the molten material and must receive its heat by conduction through the lower stratum of the layer in immediate contact with the molten bath. Therefore, I deem it preferable to work with the practical maximum rate of flow of the bath and the practical minimum thickness of fuel.

It is true that it has been experimentally determined that in the ordinary carbonizing retort the carbonization proceeds toward the center of the charge at the rate of about 1 inch per hour. Here, however, the conditions are entirely different from those which obtain in my process. The fragments of the charge in the ordinary method of carbonization are of considerable size and the charge is quiescent, the transfer of heat taking place principally by conduction from the retort walls and from the hot gases evolved from the coking coal. Radiation from the retort walls and from the highly heated layers of the charge in contact therewith also plays an important though minor part.

In my process of carbonization, which is the subject of this application, the transfer of heat takes place almost entirely by conduction from a molten substance having a very high co-efficient of conductivity. Instead of the charge being quiescent there is an active mixing or agitation of the charge due to the rapid circulation of the molten bath. As shown, the material enters the carbonizing chamber at a high velocity and in a direction transverse to the general direction of flow through the chamber. As a consequence there is a whirling or eddying movement given to the material of the bath as well as the movement of progression longitudinally of the chamber. This insures a thorough mixing and stirring up of the floating particles of coal that brings all parts of the floating blanket into direct contact with the metal of the bath.

The velocity of flow given to the bath is such as will give the coal just the proper time to become thoroughly carbonized in passing from the inlet end of the chamber 11 to the discharge end. Since the rate of flow of the bath depends, solely, upon the speed of rotation of the propeller or other circulating means, it is plain that I have a thorough and complete control over the time during which the coal is exposed to a carbonizing heat.

The temperature of distillation may, obviously, be adjusted to any point desired. It is simply a question of the temperature to which the molten material is raised in the reheater. By choosing an appropriate material for the carbonizing bath the distillation may be carried out at any desired temperature. It has been found that coal distills completely at a temperature approximating 800° Fah. When distilled at this temperature both the calorific and illuminating power of the gas obtained per unit weight of coal is much greater than that of the gas obtained from the same weight of coal distilled under the conditions that obtain in the present commercial processes of distillation.

When the carbonized coal reaches the discharge end of the carbonizing chambers it is skimmed off from the surface of the bath by the projecting ribs or paddles on the revolving drum 13 which has a shaft 14 extending through the wall of the carbonizing chamber through a suitable stuffing box 15, and having a suitable spur wheel 16, on its outer end. A suitable driving gear 17 operates the spur wheel 16, and causes the revolution of the drum 13. The coke is skimmed from the surface of the bath and raised over the dam 18 falling through the chute 19 into the water seal 20, where it is immediately quenched. The coke is withdrawn from 20 by the elevator 21. As withdrawn from the water seal the coke is often in the form of irregular aggregates of a size much larger than that of the coal particles introduced into the carbonizer. The condition of the carbonized fuel depends, however, to a great extent upon the character of the raw fuel used. With good caking coals the carbonized product is, as stated, in lumps of appreciable size. With non-caking coals the discharged carbonized coal will be, for the most part, of nearly the size charged, while with coals that decrepitate upon heating and immersion in water the discharged material may be in a thoroughly disintegrated condition. If desired, it may be used directly as a fuel for boiler firing, for instance, but I prefer to make it up into briquets before marketing it.

The gas and vapors evolved from the coal during carbonization are withdrawn from the carbonizing chamber through the pipe

22 and discharged into the hydraulic main 23 through the sealed dip-pipe 24.

The reheater 2 consists simply of a suitable furnace chamber 25, having a hearth 5 or crucible 26 for holding the molten material and a burner 27 for heating the bath. In the form of reheater shown, I use a flame of powdered fuel (preferably coke from the carbonizer 1) to accomplish the 10 heating of the molten material. Passages, 28 and 29 establish communication between the hearth 26 of the reheater 2, and the corresponding part 30 of chamber 11, below the surface of the molten material therein. 15 As shown, the circulating device is located in the passage 28. The device shown consists of a propeller 31 having a shaft 32 working in bearings 33 and 33' and having a sprocket wheel 34. A driving chain 35 20 is operated from a driving sprocket 36 on the shaft 37. It is obvious that any proper circulating means may be substituted for the one described. The molten material heated in 2 is forced through the passage 25 28 by the circulating device, a reverse current being automatically established through passage 29 from the carbonizer to the reheater. The flame from burner 27 plays along the surface of the molten bath in the 30 hearth 26 heating the metal therein and escapes from chamber 25 through the pipe 38. In the arrangement shown the products of combustion from chamber 25 are led through a recuperator for the purpose of imparting 35 their sensible heat to the current of air which is supplied to burner 27. Burner 27 need not differ materially from the devices now used in firing cement kilns. It consists of a nozzle 39, discharging through the burner 40 tube 40, and having an opening 41 through which powdered fuel is fed to the air blast by the conveyer 42. The pipe 43 conducts the hot air from the recuperator 3 to the burner 27.

45 The recuperator shown consists simply of two sets of return bend flues, one set 44, for the combustion gases from reheater 2, and another set, 45, enveloping 44, conducting the air through the recuperator.

50 Cross-flues 46 and 47 connect the several flues 44 and cross-flues 48 and 49 the separate air flues 45. The air is supplied under pressure to the flues 45 through the pipe 50 by blower 51. As shown, the combustion 55 gases are drawn through the recuperator by an exhauster 52 connected with the cross-flue 47 by the pipe 53.

In most of the present used methods of 60 making coal gas the coal is charged into chambers or retorts with comparatively thick walls of fireclay, set in suitable furnaces. The heat for the carbonization of the coal is generated in the furnaces and must be transmitted through the comparatively thick walls of the chambers or re-

torts to the charge of coal inside. This charge is usually of a thickness of several inches, about six inches in ordinary retort charging. In order to carbonize the coal in the interior of the charge the heat must pass 70 through the outer layers of the charge itself. Now coal, and more particularly, carbonized coal or coke, is an excellent non-conductor. The transfer of heat from the walls of the retort or coking chamber to 75 the interior of the charge is therefore, a very slow process. In order to avoid the necessity of allowing the charge to remain in the retorts for an undue length of time it is, therefore, necessary to maintain a 80 high temperature differential between the interior of the walls of the retort and the interior of the charge of coal therein, since the quantity of heat transmitted through a conducting medium in a given period increases with the increase in the difference 85 of temperature between the surface where the heat enters the conducting medium and the surface at which it makes its exit therefrom. Considerations of economy make it 90 necessary that the time of carbonization should be kept as short as possible. In order to properly carbonize the coal in the interior of a charge within the period of time available therefor it is necessary to 95 heat the outer layers of the charge to a temperature greatly in excess of the most advantageous temperature from a chemical point of view. The gas evolved from the interior layers of the charge must therefore pass in contact with the highly heated outer layers before it can escape from the carbonizing chamber. This results in the destruction of the bulk of the chemical combinations which were initially formed 100 in the distillation of the coal, and which are of more value than the condensable products of the secondary reactions. It is generally recognized by gas engineers that the successful distillation of coal at a comparatively low temperature, will yield products whose aggregate value is greatly in excess of the value of the products of distillation under conditions which obtain in the present processes of coal-gas manufacture. 105 The difficulty heretofore, has been that of the many proposed methods none would permit of the carrying on of the distillation of the coal at a uniformly low temperature. It is for the satisfactory solution of this problem that my invention is intended. Again, in the present method of making coal-gas in externally heated retorts, it is necessary to maintain in the furnace a temperature much in excess of that 115 of the interior of the walls of the retort itself, in order to drive the heat from the furnace through the retort walls with sufficient rapidity. Thus in order to maintain the walls of the retort at a temperature of 120 125 130

say 1800° Fah. it is necessary that the products of combustion from the furnace be permitted to escape from contact with the retorts at a temperature of about 2,000° 5 Fah. It is true that a portion of this heat may be returned to the furnace by transferring it to the air supplied for the combustion in the furnace in suitable recuperators or regenerators. In order to be sufficient such recuperators or regenerators must have a large heating surface and, therefore, not only occupy considerable space but add greatly to the cost of the apparatus required. Besides, owing to the 10 fact that the heat carrying capacity of the air is much less than the heat capacity of the combustion products and that a considerable difference of temperature must exist between the combustion products and 15 the air, in order to secure a sufficiently rapid transmission of heat through the walls of the recuperator flues, it is never possible to heat the air to the temperature of the combustion products. In retort 20 methods of gas making, therefore, the heat actually utilized in the distillation of the coal constitutes a comparatively small portion of the total heat developed in the furnace. 25 30 In my invention the heat for distillation is transmitted directly to the coal by conduction from the bath of molten substance upon which it rests. Since the coal is crushed previous to its introduction into 35 the carbonizing chamber and rests upon the molten bath in a thin sheet the distance to which the heat must be transmitted to reach the most remote particle of coal is only a fraction of an inch, whereas in the 40 present retort methods of distillation it must pass through at least three inches of fireclay and, say, six inches of the charge itself. As is well known, the retardation to heat transmission in passing from one 45 transmitting medium to another is greater than the retardation in passing through a considerable thickness of even such a poor conductor as fireclay. Therefore, by my 50 method of heating the coal by contacting it with a bath of molten material heated to the proper temperature, I secure the most favorable conditions possible for the transfer of heat to the coal undergoing carbonization. 55 Another great advantage of my method is that the evolved gas is not exposed to a temperature above that selected as the proper one for the carbonization. In the ordinary method of carbonization 60 the evolved gas is subjected to contact with the highly heated walls of the retort before it can be withdrawn therefrom. This results in secondary dissociating reactions which cause a splitting up of the carbon compounds originally formed and the forma-

tion, in general, of simpler combinations. This secondary action results in the destruction of many of the most valuable of the illuminating compounds. In my method of carbonization, on the other hand, the 70 walls of the carbonizing chamber with which the evolved gas comes into contact are heated simply by conduction from the molten bath in the hearth of the chamber. They are, therefore, at a much lower temperature than the bath itself. 75

The material which I consider best suited for the molten bath is lead. I do not, however, limit myself to the use of lead as it is manifest that I can secure the same results 80 with any suitable material which is molten at the temperature of carbonization.

I am aware that types of apparatus have been proposed before to carbonize coal by feeding the same onto a bath of molten slag 85 from smelting furnaces, or onto a bath of molten glass or similar material. Apparatus so operated, however, would necessarily produce a gas of low illuminating value and yielding but little condensable hydrocarbon, 90 owing to the relatively high temperature necessary to maintain such slag in a molten condition. As is well known, slags produced in smelting operations seldom or never attain to a condition of true fluidity below 2500° F. Ordinary iron blast furnace slag requires a temperature about 3200° to reduce it to a thoroughly fluid condition. A temperature approximating 2500° F. would cause the breaking up of practically all of the benzin and heavy hydrocarbons produced in the initially formed distillation products, as well as the ammonia and other valuable byproducts. Besides, it would be difficult to maintain a continuous 100 closed circulation of such material through separate gas-making and re-heating chambers in the manner in which I use my carbonizing bath. 105

Having described my invention, what 110 I claim is:

1. The process of carrying out the distillation of coal at a temperature below the temperature of active dissociation of illuminating constituents of the distillation products 115 of said coal to produce gas and coke which comprises continuously circulating a stream of molten metal in a closed circuit through a heating chamber and a carbonizing chamber, the said stream being heated to a temperature not above 1200° during its passage through said heating chamber whereby the temperature of distillation of said coal is maintained below that at which a substantial proportion of the distillation products 120 will be broken up, feeding crushed coal onto the stream of molten metal at approximately its place of entrance into said carbonizing chamber, maintaining said coal in contact with said stream of molten 125

130

metal during the progress of the latter through the carbonizing chamber, whereby the volatile matter of said coal is distilled therefrom, removing the fixed residue of such distillation from the stream of molten metal at the place of exit of said stream from said carbonizing chamber, removing the gaseous products of said distillation from said carbonizing chamber and subjecting them to condensation whereby the condensable constituents of said gaseous products are separated from the non-condensable constituents, substantially as described.

2. The process of manufacturing gas and carbonized materials which comprises establishing and maintaining a flowing bath or stream of molten material at a temperature not exceeding 1200° F., feeding a solid carbonaceous material containing hydrogen on and to said flowing bath, maintaining such carbonaceous material on and in contact with said bath till a desired amount of volatile material is expelled from said carbonaceous material by heat taken up from said molten material, withdrawing residual carbonaceous materials after the desired length of contact has been effected, reheating the molten material to a temperature not in excess of 1200° F. and returning the reheated molten material into contact with a fresh portion of carbonaceous material.

3. The process of manufacturing gas and carbonized fuel which comprises subjecting solid carbonaceous matter containing volatile compounds to heating by contact with a flowing bath of molten lead, said bath being maintained at a temperature such that the volatile constituents of the said carbonaceous matter are caused to be distilled therefrom but below 1200° F., and withdrawing the gases and vapors distilled from said carbonaceous material from contact with the molten lead without exposing them to a temperature that will cause the dissociation of the initial products of the distillation, substantially as described.

4. The process of manufacturing gas and producing carbonized fuel which comprises continuously circulating a bath of molten lead, or alloys of the same, first, through a heating chamber and, second, through a carbonizing chamber, feeding crushed coal onto said bath in said carbonizing chamber, contacting the said coal with the said bath during the progress of said bath through the said carbonizing chamber, whereby the volatile matter of said coal is distilled therefrom, and the carbonized residue of the coal left on the surface of said bath, removing the gaseous products of the distillation and the residual coke from said carbonizing chamber, substantially as described.

5. The process of manufacturing gas which comprises heating a bath of molten

lead, in a furnace chamber, by direct contact with a heating flame, circulating the so-heated bath through a carbonizing chamber, feeding crushed coal to the heated bath in said carbonizing chamber, whereby a portion of the heat of the bath of molten material is communicated to the said crushed coal subjecting the same to destructive distillation, withdrawing the gaseous products of the distillation and the coke from said carbonizing chamber, subjecting the said gaseous products to condensation, whereby the condensable portion of said gaseous products is separated from the non-condensable portion, withdrawing the partially cooled bath of molten lead from said carbonizing chamber and returning it to said furnace chamber, reheating said bath of molten lead in said furnace chamber and returning the so reheated bath of molten lead to the said carbonizing chamber for heating another portion of coal, substantially as described.

6. The process of manufacturing gas which comprises continuously circulating a stream of molten lead in a closed circuit through a heating chamber and a carbonizing chamber, feeding crushed coal onto the stream of molten lead at its place of entrance into said carbonizing chamber, contacting said coal with said stream of molten lead during the progress of the latter through the carbonizing chamber, whereby the volatile matter of said coal is distilled therefrom, removing the fixed residue of such distillation from the stream of molten lead at the place of exit of said stream from said carbonizing chamber, removing the gaseous products of said distillation from said carbonizing chamber and subjecting them to condensation, whereby the condensable constituents of said gaseous products are separated from the non-condensable constituents, substantially as described.

7. The process of carrying out the distillation of coal at a temperature below the temperature of dissociation of the illuminating constituents of the distillation products of said coal, which comprises continuously circulating a stream of molten lead in a closed circuit through a heating chamber and a carbonizing chamber, the said stream being heated to a temperature not exceeding 1200° during its passage through said heating chamber, feeding crushed coal onto the stream of molten lead at its place of entrance into said carbonizing chamber, contacting said coal with said stream of molten lead during the progress of the latter through the carbonizing chamber, whereby the volatile matter of said coal is distilled therefrom, removing the fixed residue of such distillation from the stream of molten lead at the place of exit of said stream from said carbonizing chamber, removing the

gaseous products of said distillation from said carbonizing chamber and subjecting them to condensation, whereby the condensable constituents of said gaseous products are separated from the non-condensable constituents, substantially as described.

8. The process of manufacturing gas and producing carbonized material which comprises contacting carbonaceous matter containing hydrogenous compounds with an advancing stream of molten material containing lead, until the said carbonaceous matter has been carbonized to the desired degree, withdrawing the resulting gas and carbonized material from contact with said stream of molten material, re-heating said molten material to a temperature that is substantially below the dissociation temperature of the illuminating constituents of the distillation products of said coal and reusing the same, substantially as described.

9. The process of subjecting coal to distillation to produce volatile products and coke which comprises feeding the said coal in comparatively small fragments onto the surface of an advancing stream of molten material maintained at a temperature below that at which water will react with carbon to form water gas, contacting the said coal with the said molten material until carbonization has been effected and then removing the residual coke from contact with said molten material, substantially as described.

10. The process of subjecting coal to distillation to produce volatile products and coke which comprises feeding the said coal onto the surface of an advancing stream of molten material to form a comparatively thin layer on the surface of said stream, whereby the said coal is heated by direct conduction from the said molten material and the volatile matter of said coal distilled therefrom, and removing the fixed residue from such distillation from the surface of the said molten material, when the said distillation has progressed to the point desired, substantially as described.

11. The process of distilling coal to produce volatile products and coke which comprises continuously feeding coal onto an advancing stream of molten material contained in an inclosed chamber, the said coal being fed onto the said stream at substantially its place of entrance to said chamber in a comparatively thin layer whereby the said coal is heated chiefly by direct conduction of heat from said molten material and its volatile matter distilled, causing the said coal to be borne through said chamber by said stream of molten material, and removing the fixed residue of such distillation from said molten material at substantially its place of exit from said chamber, substantially as described.

12. The process of distilling coal to pro-

duce volatile distillation products and coke which comprises continuously feeding coal onto a stream of molten material flowing through an inclosed chamber, the said coal being fed onto the said stream at substantially its place of entrance to said chamber, causing said coal to be borne through said chamber on the surface of said stream of molten material and removing the products of the distillation of said coal from said chamber in proximity to the place of exit of said molten material from said chamber, whereby the said distillation products are withdrawn from said chamber without exposing them to a temperature higher than that at which said coal was distilled, substantially as described.

13. The process of distilling carbonaceous material containing volatilizable constituents to produce distillation gases and coke, which comprises continuously feeding the said carbonaceous material in a relatively thin layer onto the surface of a stream of molten material flowing through an inclosed chamber, whereby the said carbonaceous material is quickly heated to a carbonizing temperature by direct conduction of heat from said molten material, causing said coal to be transported through said chamber on the surface of said stream of molten material and continuously removing the coked residue from the distillation of said carbonaceous material at a place approximately the point of exit of said molten material from said inclosed chamber, substantially as described.

14. The process of distilling coal which comprises heating a stream of molten material by directly contacting the same with hot combustion gases, forcibly injecting the so-heated molten material into an inclosed carbonizing chamber, the said molten material being injected into the said inclosed chamber at such an angle to the axis of said chamber that a vortex is created in the said stream of molten material, continuously feeding into said vortex crushed or otherwise formed fine coal, whereby the particles of said coal are immediately brought into intimate contact with the said molten material and quickly heated to a distilling temperature, continuously withdrawing said molten material from the extremity of said carbonizing chamber opposite to that at which it was introduced thereinto, whereby the said molten material is caused to flow from end to end thereof, thereby transporting the said coal through said carbonizing chamber while the said coal is undergoing carbonization, and continuously removing the carbonized residue of said coal from the extremity of said carbonizing chamber opposite to that at which it was introduced, substantially as described.

15. The process of distilling coal which

comprises heating a stream of molten material to a temperature below 1200° Fah. by directly contacting the same with hot combustion gases, forcibly injecting the so-heated molten material into an inclosed carbonizing chamber, the said molten material being injected into the said inclosed chamber at such an angle to the axis of said chamber that a vortex is created in the said stream of molten material, continuously feeding into said vortex crushed, or otherwise produced, fine coal, whereby the particles of said coal are immediately brought into intimate contact with the said molten material and quickly heated to a distilling temperature, continuously withdrawing said molten material from the extremity of said carbonizing chamber opposite to that at which it was introduced thereinto, whereby the said molten material is caused to flow from end to end of said chamber, thereby transporting the said coal through said carbonizing chamber while the said coal is undergoing carbonization and continuously removing the carbonized residue of said coal

from the extremity of said carbonizing chamber opposite to that at which it was introduced thereinto, substantially as described.

16. The method of subjecting coal to quick distillation at a relatively low temperature which comprises heating a bath of molten material to a temperature of between 800° and 1200° Fah., creating a vortex in said bath and continuously feeding crushed coal into said vortex whereby the particles of said crushed coal are immediately brought into contact with the material of said bath and are quickly heated to the temperature of distillation by direct conduction of heat from said molten material, substantially as described.

Signed at New York city in the county of New York and State of New York this 23rd day of Dec. A. D. 1909.

HENRY L. DOHERTY.

Witnesses:

W. J. QUENTIN,  
W. G. BERRYMAN.